

# UNITED STATES PATENT OFFICE.

GEORGE D. VAN ARSDALE AND CHARLES G. MAIER, OF NEW YORK, N. Y.

## METHOD OF ELECTROLYTICALLY PRECIPITATING METALS AND COMPOUNDS FROM SOLUTIONS.

1,371,826.

Specification of Letters Patent. Patented Mar. 15, 1921.

No Drawing.

Application filed May 13, 1918. Serial No. 234,241.

To all whom it may concern:

Be it known that we, GEORGE D. VAN ARSDALE and CHARLES G. MAIER, citizens of the United States, and residents of New York city, in the county of New York and State of New York, have invented certain new and useful Improvements in Methods of Electrolytically Precipitating Metals and Compounds from Solutions, of which the following is a specification.

This invention is an improvement in methods of electrolytically precipitating metals and compounds from solutions.

It is applicable to those processes in which an insoluble anode is used and in which the metal to be recovered is deposited at the cathode, also to processes in which a compound of a metal is separated at the anode and hydrogen evolved at the cathode, and is finally of very considerable advantage if utilized in cases where two ores of certain kinds are to be treated together.

In the first two cases the use of depolarizing agents is known, but in most cases such depolarization results in the accumulation in solution of the products of depolarization with detriment to further electrolytic efficiency. The improvement which we have made, and which may be applied in a variety of ways, is the use of depolarizers, the products of whose depolarizing action are insoluble and therefore do not accumulate in solution, and which also may be recovered by reason of this fact and re-used cyclically in subsequent operations. We have also found several cases in which two products, which are to be recovered, may be so recovered by electrolysis at the same time in the same cell, one at the anode and one at the cathode, and in which operation they act mutually as depolarizing agents, giving a reduction in voltage and consequent economy in power.

Several special cases in which this invention may be applied are described, but others will be mentioned only, and others again will occur to those skilled in the art, all of which employ this discovery.

In the electrolytic precipitation of copper from solution using insoluble anodes, as a part of a leaching process for separating copper from ore, it has been found desirable to use depolarizing agents, both for the purpose of reducing the voltage otherwise needed, and also for the purpose of prevent-

ing anode disintegration which otherwise occurs to a prohibitive degree in the electrolysis of sulfate solutions. Iron salts and sulfur dioxide have been proposed and used separately or in combination for such purposes. Iron, however, is open to some objection since although ferrous sulfate is an efficient anodic depolarizer, the product of its depolarizing action, ferric sulfate, accumulates in the solution during the electrolysis, and rapidly reduces the cathodic efficiency, the practical result being that only a small portion of the copper present can be efficiently precipitated at each cycle.

The solution must then be withdrawn from the electrolysis and the ferric iron reduced, or reduction of the ferric iron must be done during the electrolysis both of which are more or less inconvenient. The present invention provides a means for accomplishing both of the above purposes in the electrolysis of solutions of copper, namely depolarizing and reduction of voltage, and prevention of disintegration of anodes, and the result of this depolarizing action is a solid product precipitated at the anode. As a consequence of this fact there is no accumulation of the depolarizing product in the solutions, as when iron is used which is evidently of great practical importance. Also the same depolarizer may be used cyclically as described later.

Our present invention, however, is not only of advantage in this respect as indicated above, and as will be described later, but is also of advantage in the electrolysis of solutions of manganese to produce manganese dioxide and free sulfuric acid as a part of processes for extracting manganese from its ores. Methods for accomplishing this have been described, which consist essentially in the leaching of manganese ores by suitable reagents to produce manganese sulfate solutions, and the subsequent electrolysis of such solutions, making manganese dioxide at the anode and free sulfuric acid in the electrolyte. Such a process is satisfactory, but is open to the objection that the voltage is high, differing from the high voltage in copper electrolysis above mentioned, in that in this case we are concerned with the reactions at the cathode instead of at the anode. In other words what is needed for a more economical electrolytic production of manganese dioxide is a cathodic de-

polarizing agent, and we have discovered that copper in solutions of manganese will act very efficiently as such a cathodic depolarizer, which is evidently of advantage 5 in that less power is required per unit of manganese. By combining and utilizing together both of these depolarizing agents at the cathode and the anode, we have discovered a method of simultaneously producing, by electrolysis, copper and manganese dioxide from the same solution at relatively low voltages and good efficiencies, and also with freedom from anode disintegration and with the further advantage that there 10 15 is no accumulation in the solution of the result of depolarization at either electrode as in other methods of electrolyzing with depolarizing agents.

It is evident that this invention is of value 20 as a part of processes for extracting either manganese or copper or both from their ores either together or separately.

It can be seen that our invention can be utilized in a number of ways, several of 25 which are mentioned and described below. For example, in the recovery of manganese and copper from ores there are three cases—(1st) in which it is desired to treat a manganese ore alone for the recovery of manganese; (2nd) in which it is desired to treat a copper ore alone for the recovery of copper; and (3rd) in which it is desired to treat both manganese and copper ores together for the recovery of both manganese and copper. 30 35 40 45 In all three cases the invention used is the same but the manner of use differs as follows. In the first case above, the copper as sulfate is used cyclically in the recovery of manganese which is removed and marketed; in the second the manganese is used cyclically in the recovery of copper which is removed and sold; and in the third both manganese and copper act mutually as depolarizing agents and are both removed and sold.

In all three cases the products of depolarization are insoluble, solid products, produced at the electrodes and not, as in other electrolytic processes, in which depolarization is used, soluble products which accumulate in the electrolyte and by their presence proportionally reduce deposition efficiencies.

One way in which each of the above three possibilities may be carried out for recovering copper and manganese, will now be described.

For the first case it is assumed that there is a supply of manganese ore suitable for leaching and electrolytic recovery of manganese, but no available supply of suitable copper ore. The manganese ore is treated so as to obtain a substantially pure solution of manganese sulfate, which may be done as follows: The ore is crushed and suspended in water, to which, if necessary some acid

is added, and agitated in a suitable device. During agitation  $\text{SO}_2$  is passed into the pulp and agitation and passing of  $\text{SO}_2$  are continued until all of the soluble manganese is in solution. Carbonate or other than dioxide ores of manganese may also be treated by dissolving the manganese by the sulfuric acid produced during the subsequent electrolysis, or by acid added from outside sources. The solution and residue are then separated 75 and the solution treated to remove iron, thionates or other compounds objectionable in electrolysis.

This may be done in several ways. The amount of thionates produced in leaching 80 manganese from its ores by sulfur dioxide will be greatest in cold, neutral solutions, and least in hot, acid solutions. With a solution between 60° and 100° C. and containing from 5% to 10% free sulfuric acid, the amount of 85 thionates will not be enough to interfere with subsequent operations. The solution is then placed in contact with a fresh amount of dioxide manganese ore, without adding  $\text{SO}_2$ . This is for the purpose of oxidizing any iron 90 present to the ferric condition, and also for oxidizing any remaining thionates. The object of changing the iron to the ferric condition is because iron in the ferrous greatly reduces the current efficiency of anode deposition of  $\text{MnO}_2$ . The ferric iron produced 95 may be enough to interfere with the deposition of copper at the cathode, but this is not important for this particular application of the process, since being entirely in the 100 ferric condition it may be precipitated and removed.

A solution of copper sulfate is then added to the solution of manganese sulfate, the copper sulfate being obtained as described 105 later. The solution should contain an amount of copper chemically equivalent to the amount of manganese subsequently separated by the electrolysis, at the anode. The solution containing copper and manganese is 110 then preferably heated to between 60° and 70° C., and subjected to electrolysis while hot. The usual electrodes and apparatus employed for this purpose may be used. We prefer to use carbon, graphite or coke as 115 anode material, and as cathodes either copper or iron sheets. The current density may be at any commercially economical point, say six amperes per square foot or more. If the current density 120 is high enough, for example about twenty amperes per square foot, a part or all of the deposited copper will be in a spongy form, and therefore more readily detached and oxidized later. The object of this 125 is so that it may be thus readily oxidized later. If copper were not present the electrolysis of manganese sulfate solution alone would produce manganese dioxide at the anode and free sulfuric acid in the electro- 130

lyte, but the voltage would be high, and hydrogen would be evolved at the cathode. When copper is present under exactly the same conditions no hydrogen is evolved at 5 the cathode, copper being deposited instead, and the result is a considerable decrease in the voltage. After electrolysis has proceeded for a sufficient length of time, depending on the anode and cathode efficiency obtained and the use to which the manganese 10 dioxides and acid produced are to be put, the electrolyzed solution is separated from the dioxides and the latter separated from the anode or otherwise treated and prepared for 15 use as described elsewhere, and fresh portions of original electrolyte are again prepared and subjected to electrolysis, the process being thus made continuous. A portion of the acid produced may be used for 20 treating the ore in case all of the manganese is not soluble, by means of  $\text{SO}_2$ , or acid from an outside source may be added.

During the electrolysis of the solution, as stated above, copper is precipitated at the 25 cathode. If this is precipitated in a spongy form it may be readily detached from the cathode, and is then easily oxidized by heating or otherwise, and after oxidation is then dissolved in a portion or all of the acid 30 resulting from the electrolysis. The solution thus made may then be used for suspending the crushed manganese ore for the first stage of the process as described above. Variations in the above procedure may of 35 course be made if desired, using the same principles.

For the second case it is assumed that there is a supply of copper ore suitable for leaching, but no available supply of manganese 40 ore in large amounts. In this case the manganese dioxide produced is used cyclically as the depolarizing agent, and the copper becomes the main product to be disposed of, differing from the first case in which the copper 45 is used cyclically.

Operation may be as follows: The copper ore, in which the copper may be either in the oxidized or sulfid state, is leached by a solution in which the active leaching agents are 50 sulfuric acid and ferric sulfate, and which also contains manganese sulfate. This may be done in any suitable apparatus, preferably some form of counter-current leaching device. The sulfids present will reduce 55 a part or all of the ferric iron to the ferrous condition. This ferrous iron is objectionable in the subsequent electrolysis and is therefore oxidized to the ferric state, which is accomplished by the  $\text{MnO}_2$  produced subsequently. If the ferric iron is 60 present in too large an amount a portion of it may be removed by precipitation at this point. The ferric iron produced is not so objectionable for electrolysis and production of copper as in the usual methods, since

under the conditions of our work a high current density may be employed and a high cathodic deposition efficiency obtained even in the presence of considerable ferric iron. The solution is now subjected to electrolysis 70 in apparatus arranged for continuous operation. The copper deposited at the cathode is withdrawn from time to time and treated in the same way as electrolytic copper from other electrolytic processes. 75

The manganese dioxide precipitated at the anode from the manganese sulfate present in the solutions, is also removed from time to time. It is unnecessary to detach this from the anodes, since it is used to oxidize  $\text{Fe}^{+2}$  to 80  $\text{Fe}^{+3}$  and since  $\text{MnO}_2$  is very readily soluble in very weak, acid solutions of ferrous iron, being thereby dissolved and returned to the cycle as described above.

The solution resulting from the electrolysis will contain ferrous and ferric iron, free acid and any residual copper and manganese.

The current density at the cathode during electrolysis having been maintained sufficiently high to overcome the dissolving action of ferric iron on the copper deposited, and a good efficiency having thus been obtained, the resulting solution will have most of its iron in the ferric condition. 90

It is desirable for the subsequent leaching which is done with this solution, to have all of the iron in the ferric state, and this may be done by using a part of the deposited  $\text{MnO}_2$  for this purpose, the result being an 100 acid solution with all iron as ferric iron, which is now applied to a fresh portion of ore and the process thus repeated.

For the third case it is assumed that we have available supplies of both copper and manganese ores, suitable for leaching. In the copper ores it is immaterial whether the copper is present as oxid or sulfid. It is important that at least a large amount of the manganese be in the form of dioxide in its 110 ore. Whether acid in addition to that provided by the cycle of operations will be needed or not, depends on the acid consuming character of the ores being treated. If extra acid is needed it may be produced by 115 an additional step of the process to be described later, and as much as required may be made in this way.

The manganese and copper ores to be leached may be treated either together in the 120 same apparatus or separately. We prefer to treat them together, and as before in apparatus suited for counter current leaching.

The solution for leaching will contain amounts of sulfuric acid and ferric iron 125 equivalent to the amount of copper and manganese electrolytically deposited, and any copper and manganese remaining after electrolysis.

The copper and manganese ores being 130

treated are brought into contact with this solution whereby their copper and manganese values are brought into solution, and the resulting solution is then separated from the tailings, which are preferably washed before being discarded.

If the amount of iron in the solution thus obtained is too great for proper electrolysis, it may be readily removed by precipitation or otherwise and the accumulation of impurities may also be provided for at this point by the removal altogether of a part of the solution and the treatment of this for the recovery of its values by other methods.

The solution is now subjected to electrolysis, which is done in the usual form of apparatus, arranged for continuous operation, at current density equivalent to six amperes per square foot or more. There will be produced copper at the cathode, and manganese dioxid at the anode, both of which are removed from the tanks from time to time. The copper is deposited on starting sheets made in the usual way, and the cathodes produced are treated the same as cathodes from other electrolytic methods. The manganese may be deposited on graphite or carbon anodes, and subsequently removed from them as described elsewhere, or crushed coke or carbon may be employed as anode material. The electrolysis is continued as long as reasonable cathode and anode efficiencies are obtained.

The resulting solution may not contain enough free acid for the subsequent treatment of fresh amounts of ore, and if so a part or all of the ferric iron present may be reduced by sulfur dioxid, making equivalent amounts of free acid and ferrous iron, the latter being again oxidized to ferric iron by adding ore containing manganese dioxid at this point. The solution thus treated is separated from the residue of the manganese ore and will then have all of its iron in the ferric state and be thus available for repeating the process on fresh ores.

It is evident that by the repetition of this last step as much free acid as required may be made at the expense of an accumulation of manganese.

The above special applications of the process have been fully described. There are in addition a number of other ways in which the same principles may be utilized. Generally speaking the soluble salt of any metal capable of forming a metallic compound at the anode, the metal in which is in a higher state of oxidation than it was previously when in solution, may be used as an anodic depolarizing agent with the described advantages in the electrolytic separation of a metal from solution. Other examples of such metals capable of thus acting under proper conditions are lead, vanadium,

etc. Generally speaking also in the recovery of such metals as last mentioned, by separation at the anode the soluble salt of the same or another metal capable of giving a metallic deposit at the cathode instead of the hydrogen which would otherwise be evolved, may be used as a depolarizer. And finally, combinations of the depolarizing action at both electrodes as described in the above special case may be used.

Having thus described the invention, what is claimed as new is:—

1. An improved method of depolarization in electrolysis which comprises the cyclical use as a depolarizing agent of a metal, a soluble salt of which is capable as a result of electrolysis, of yielding a metal or metallic compound at an electrode, and removing said metal or metallic compound and treating the same to regenerate the salt of the metal originally used as a depolarizing agent in subsequent electrolysis.

2. An improved method of electrolysis which comprises in electrolyzing a solution containing a copper salt capable of producing an insoluble deposit at one electrode, while a metal or compound is produced at the other electrode, removing said deposit, treating the deposit to regenerate the original compound, and using this regenerated compound for subsequent electrolysis in the same way cyclically.

3. An improved method of depolarization in electrolysis which comprises the cyclical use as a depolarizing agent of copper, a soluble salt of which is capable, as a result of electrolysis, of yielding copper or a copper compound at an electrode, removing said copper or copper compound being removed and treating the same to regenerate the copper salt originally used as a depolarizing agent in subsequent electrolysis.

4. The process of producing copper from its ores which comprises leaching an ore of the metal with a solution containing sulfuric acid, ferric sulfate, and a salt of an electro-positive metal, and electrolyzing the solution whereby to obtain a deposit of copper in the metallic state at the cathode, and a deposit of the electro-positive metal or an insoluble compound thereof at the anode.

5. The process of producing copper from its ores which comprises leaching an ore of the metal with a solution containing sulfuric acid, ferric sulfate, and a salt of an electro-positive metal, electrolyzing the solution whereby to obtain a deposit of copper in the metallic state at the cathode, and a deposit of the electro-positive metal of an insoluble compound thereof at the anode, removing the anode deposit, and treating the same with the solution which results from the step of electrolysis whereby to regenerate the salt of the electro-positive metal originally employed, whereby the

same may be used cyclically as a depolarizing agent.

6. The process of separating metal values from a composite solution containing an electro-negative metal and an electro-positive metal, by a process of electrolysis which comprises leaching ores of the two metals with a solution of sulfuric acid, and, if required, ferric iron, and electrolyzing the 10 solution whereby to obtain a cathodic deposit of the electro-negative metal and an anodic deposit of the electro-positive metal, and in which step of electrolysis the metals mutually act as depolarizing agents.

7. The process of producing copper in the 15 metallic state and manganese dioxide from a composite solution of sulfates of these metals which comprises subjecting such composite solution to electrolysis and thereby effecting an anodic deposition of manganese dioxide and a cathodic deposition of copper in the metallic state. 20

Signed at New York in the county of New York and State of New York this 17th day of April, A. D. 1918.

GEORGE D. VAN ARSDALE.  
CHARLES G. MAIER.